

# UNITED STATES PATENT OFFICE.

WILLIAM E. GARDNER, OF PITTSBURGH, PENNSYLVANIA, ASSIGNOR OF ONE-THIRD TO  
HENRY CLAY BLACK, OF BEN AVON, PENNSYLVANIA, AND ONE-THIRD TO JULIUS  
JACOB, OF PITTSBURGH, PENNSYLVANIA.

## ELECTRICAL-HEATER RESISTANCE ELEMENT.

1,338,294.

Specification of Letters Patent.

Patented Apr. 27, 1920.

No Drawing.

Application filed July 7, 1919. Serial No. 309,133.

*To all whom it may concern:*

Be it known that I, WILLIAM E. GARDNER, a resident of Pittsburgh, in the county of Allegheny and State of Pennsylvania, have 5 invented a new and useful Improvement in Electrical - Heater Resistance Elements, of which the following is a specification.

The invention relates to electrical resistance elements and more particularly to resistance elements for electrical heaters or radiators.

The object of the invention is to provide a resistance element of the character described which will not burn out, which remains practically unchanged no matter how 15 long used, and which nevertheless is cheap to produce and economical to use.

In general the invention consists in a resistance unit composed of non-metallic, non-fusible and non-combustible substances under the heating current. More specifically, 20 it comprises an electrical resistance element formed of a mixture of finely divided non-metallic conducting and non-conducting substances, which will not fuse and therefore remain in their original condition no 25 matter how long used.

Various substances can be used for the two elements of the compound. As the conducting element of the compound I prefer 30 to use carbon, and preferably that form of carbon found in substantially pure coke. For the non-conducting element of the compound various substances can be used, preferably 35 bone ash or bone earth, such as can be obtained on the market in various grades,—that which is best for my purposes being the white bone ash; or commercial carborundum may be used as the non-conducting element. These ingredients will be 40 mixed in a finely divided state, either granulated, but preferably in powdered form. The finer the ingredients the better, as it obviates any slight arcs which might form 45 between the grains of granulated material. Satisfactory results are secured by reducing the ingredients to a size to pass through a sixty-mesh sieve or finer.

These ingredients reduced to a fine state 50 are then very thoroughly mixed, so that all the particles of the conducting material (carbon) are divided or separated by particles of non-conducting material (bone ash

or carborundum, or both). The more intimate the mixture the better the result. 55

The proportions of the ingredients may be varied, depending upon the particular use to which the heater is to be applied, and to the voltage and amperage of the current to which it is to be subjected. With high 60 voltage currents obviously the proportion of the non-conducting or insulating ingredient must be greater than for a low voltage current. Likewise the higher the resistance of the non-conducting ingredient the less the 65 amount that need be used. In general I have found that carborundum must be used in a slightly larger proportion than bone ash, as carborundum is not as good an insulator as bone ash. For ordinary purposes 70 I have found that a mixture consisting of three parts of carbon to one part of bone ash (or a slightly greater amount of carborundum when the latter is used in place of bone ash) gives satisfactory results. 75

This composition can be used either in a loose dry form or can be formed into a solid by the use of a suitable binder. It can be used in loose dry form by merely placing it in a tube composed of electrically non-conducting but heat conducting material, or in a metallic tube provided with a suitable electric insulating lining and having the two terminals of the electric circuit inserted into the ends of the tube and into the powdered 85 material; or such dry material may merely be placed in an electric non-conducting pan or trough, such as one composed of porcelain or earthen ware, with the terminals of the circuit inserted into the powdered material at opposite ends of said pan or trough. It can also be molded into solid form of any desired size or shape by the use of a binder which is non-fusible under the heating current and which does not form too high a 90 conductor of electric current. I have found that if these dry ingredients are mixed with a very small quantity of molasses and then molded and carbonized at a high heat in a closed receptacle a very solid and durable 95 resistance element is formed. 100

These resistance elements can be connected in the circuit either in multiple arc or in series or in any other well known way of connecting elements in an electric circuit. 105 They can be made of any desired size or

length. In general for a current of given value, resistance elements of different lengths can be used by varying the relative amounts of conducting and none-conducting ingredients. That is to say, the longer the element (that is, the longer the distance the current must travel through the resistance element between the electrical terminal) the larger should be the percentage of conducting material relative to the non-conducting material.

A resistance element composed of the ingredients specified is cheap to produce, is highly efficient in use, does not burn out as do metallic resistance elements, and furthermore is practically unaffected by the electric current due to the fact that the elements do not fuse together under a heating current but always remain in the condition of original mixture.

This resistance element can be used for any purpose or in any place where an electrical resistance element for heating purposes can be used.

Obviously various kinds of ingredients suitable for the purpose stated will suggest themselves to those skilled in the art. Likewise the proportions of these ingredients can be varied within quite wide limits, depending upon the characteristics of the specific ingredients used, the value of the current of the circuit in which the same is to be inserted, and the particular use to which the heating element is to be put.

I claim:

1. An electrical resistance element consisting of an intimate mixture of finely divided dry carbon, and finely divided bone ash.
2. An electrical resistance element consisting of an intimate mixture of finely divided coke, and finely divided bone ash.

In testimony whereof I have hereunto set my hand.

WILLIAM E. GARDNER.

Witness:

G. G. TRILL.